

## UNITED STATES PATENT OFFICE

1,976,803

## COPPER ALLOY

William B. Price, Waterbury, Conn., assignor to  
Scovill Manufacturing Company, Waterbury,  
Conn., a corporation of Connecticut

No Drawing. Application February 28, 1934,  
Serial No. 713,265

## 3 Claims. (Cl. 75—1)

This invention relates to a copper alloy and it has for its object to provide an alloy which will be resistant to corrosion cracking and season cracking, unaffected by mercury or compositions containing mercury, capable of being cold drawn and cold worked with a greater reduction of area and much higher tensile strength than has heretofore been obtained, while still retaining a good elastic limit, thus making the alloy especially suitable for withstanding high pressures so that it serves admirably for cartridge cases and shot gun shells for modern high pressure explosives. Of course, it may also be readily worked hot and is suitable for many purposes when so worked, as it still retains its resistance to corrosion cracking and season cracking, but when worked cold, or if hot worked first and then worked cold, without any annealing or heat treatment, an extreme hardness and strength may be obtained. While it can be so worked that it is harder and of greater strength than copper, it is very ductile and tough.

With the above object in view, the invention consists in adding to copper a rather small percentage of silicon, tin and iron, the percentages ranging as follows:

|                               | Per cent     |
|-------------------------------|--------------|
| Silicon                       | 0.1 to 1.00  |
| Tin                           | 0.01 to 0.50 |
| Iron                          | 0.01 to 0.75 |
| Balance substantially copper. |              |

It is to be understood that impurities must be kept as low as is commercially possible, or the valuable properties of the alloy will be injuriously affected. The ingredients may be combined in any of the usual metallurgical ways, for example, the copper may be melted first, then the iron and silicon added separately or combined as a ferro-silicon compound and finally the tin added to the molten mixture. Instead of this the tin and ferro-silicon may be added simultaneously to the molten copper, or all the ingredients may be put together cold and the whole then melted.

Two compositions which give the best results are as follows:

## No. 1

|                 | Per cent |
|-----------------|----------|
| Silicon         | 0.5      |
| Tin             | 0.25     |
| Iron            | 0.25     |
| Balance, copper | 99.00    |

## No. 2

|                 | Per cent |
|-----------------|----------|
| Silicon         | 1.00     |
| Tin             | 0.25     |
| Iron            | 0.25     |
| Balance, copper | 98.50    |

60 The second alloy above set forth is capable of

being worked cold to give a somewhat harder material than the alloy lower in silicon.

With all of the alloys of the present invention the ductility is high when high hardness is obtained, and most important of all is the great 65 increase in tensile strength, a result not heretofore obtainable with copper alloys suitable for cartridge metal. Although iron is present it is in such a small percentage and its action is so modified by the other metals that it has no injurious effect on the cartridge cases such as has been considered objectionable with copper alloys containing iron.

The alloys above described can be readily worked into seamless tubes and pipes, which is 75 not so easily done with alloys having higher percentages of silicon, iron and tin, yet the final product maintains the other valuable properties of such compositions.

A further important feature of the alloy is 80 that it may be welded by any of the modern welding systems, such as the gas or electric welding methods. Also the alloy may be made into welding rods which are suitable for welding not only the same kind of alloy material but other 85 types of copper alloys and the weld metal is particularly satisfactory on account of its high strength and resistance to corrosion of the kinds usually encountered in practice and to season cracking, thereby providing a permanent weld. 90

Having thus fully described the invention, what I claim is:

1. A copper alloy having a composition within substantially the following range:

|                                | Per cent     |
|--------------------------------|--------------|
| Silicon                        | 0.1 to 1.00  |
| Tin                            | 0.01 to 0.50 |
| Iron                           | 0.01 to 0.75 |
| Balance, substantially copper. |              |

2. A copper alloy having substantially the following composition:

|                 | Per cent |
|-----------------|----------|
| Silicon         | 0.5      |
| Tin             | 0.25     |
| Iron            | 0.25     |
| Balance, copper | 99.00    |

3. A copper alloy having substantially the following composition:

|                 | Per cent |
|-----------------|----------|
| Silicon         | 1.00     |
| Tin             | 0.25     |
| Iron            | 0.25     |
| Balance, copper | 98.50    |

WILLIAM B. PRICE.

115

120